

## UNITED STATES PATENT OFFICE

2,574,994

## LUBRICATING COMPOSITION

David E. Adelson, Berkeley, Calif., assignor to  
Shell Development Company, San Francisco,  
Calif., a corporation of Delaware

No Drawing, Application October 24, 1947,  
Serial No. 782,045

11 Claims. (Cl. 252—46.6)

1

This invention relates to novel reaction products having properties of greatly improving and stabilizing lubricants. The invention also pertains to lubricants, such as mineral lubricating oils, synthetic lubricants of hydrocarbon or non-hydrocarbon origin, and the like, containing a multi-functional additive having detergent and anti-ringsticking properties, which additive also acts as an inhibitor of oxidation and corrosion.

It is well known that various lubricants, whether doped or undoped, tend to oxidize and to form corrosive bodies and sludge, when used in modern engines and machines operating under ordinary conditions or at high speeds, elevated temperatures, heavy loads and/or other adverse conditions. Some of the deterioration products of lubricants formed during their use are hard carbonaceous materials which adhere to metal surfaces and cause scratching and scuffing of movable metal parts, as well as the sticking of valves and piston rings in engines. In addition, the known lubricants are generally incapable of maintaining a continuous lubricating film between movable metal parts; therefore, their use results in gradual or even rapid wear of metal parts. The damage thus caused requires replacement of such parts or even the complete overhauling of engines and machines, thus resulting in expensive loss of production and time.

In the case of the highest quality non-corrosive, stable lubricating oils, which have been highly refined, or synthetic lubricants developed for specific or special uses, it has been observed that such oils or lubricants are generally highly susceptible to oxidation and deterioration, becoming progressively more corrosive when used in engines and machines even under ordinary operating conditions.

To improve the lubricating properties of mineral oils and synthetic lubricants it has become the practice to incorporate into these various lubricants at least one and in most cases more than one addition agent, which additives have the effect or property of inhibiting deterioration of lubricants and impart to them certain beneficial properties. Thus, additives have been specifically developed to have the property of inhibiting corrosion of alloyed bearings such as copper-lead, cadmium-silver and the like, used in automotive, diesel and aircraft engines. Acidic oxidation or decomposition components formed in lubricants during use readily attack these bearings but are inhibited or prevented from effecting such deterioration by the formation of a corrosion protective film on the bearing surface. Additives have also been developed which possess the property of modifying the carbonaceous materials formed (by deterioration of lubricants) on piston rods, rings and valves, and other metal parts in internal combustion engines, automotive and

2

truck engines, aviation engines, high speed diesel engines, and the like. Such additives serve a very important function because, by modifying this carbonaceous material so that it can be readily removed, the tendency of engine parts to become stuck is inhibited so that ringsticking, piston scuffing, scratching and wearing away of other engine parts, and a material reduction of engine efficiency, are prevented or materially inhibited.

10 Other additives have been developed for the purpose of acting as detergents in lubricants in order to assist in the removal of soot, sludge, varnish, and/or lacquer, formed from deterioration of the oil when subjected to high operating temperatures. Detergents, due to their cleaning action, prevent the accumulation of these deleterious materials and assist in removing those which are formed.

Anti-wear additives have the property of reducing friction of movable metal parts of the same or different metals. Due to the function exerted or property imparted by such additives to lubricants, wear caused by direct frictional contact of metals can be greatly reduced. Also, 15 additives have been developed to withstand extreme pressures, disperse impurities, solubilize certain additives and the like.

The development of the large number of various additives has been due to the fact that most, 20 if not all such additives are capable of functioning in substantially only one specific manner. Very few lubricant additives have the ability of improving a lubricant in more than just one respect. Thus, a good anti-oxidant might not be able to inhibit lacquer and varnish formation on piston rods, or to act as a detergent or corrosion inhibitor. In many cases it is found that an additive possesses very good properties in one respect, but is detrimental as an additive in another respect. Therefore, the use of still other additives is frequently required to obtain a relatively good stable lubricant. The combination of additives in lubricants wherein each additive exerts its influence without interfering with the 25 function of other additives is a difficult matter to attain. In most cases, additives co-react or interfere with each other. To prevent this, great care must be taken in selecting the additives, mixing them in specific proportions, and continuously watching and replacing additives which have stopped functioning or have deteriorated.

It is an object of this invention to improve the lubricating properties of various lubricating bases by the addition thereto of a minor amount 30 of a multi-functional material. Another object of this invention is to add to compounded or doped lubricants a multi-functional material whereby a synergistic effect is produced, resulting in a product of accentuated and improved properties. Another object of this invention is

to add to oleaginous materials, mineral lubricating oils, synthetic lubricants and the like, a multi-functional material so as to inhibit oxidation and corrosion and prevent the formation of sludge, varnish and lacquer in said lubricants even under adverse operating conditions. Still another object of this invention is to use in lubricating compositions, a multi-functional material which prevents ringsticking as well as the sticking of other engine parts due to deterioration of the 10 lubricant. Also it is an object of this invention to use in oleaginous materials, e. g. in lubricating compositions, a multi-functional material which inhibits wear, scuffing, scratching and other damage to engine parts. Furthermore, it is an object 15 of this invention to provide novel multi-functional improving and enhancing additives for lubricating bases. Other objects of this invention will appear as the description proceeds.

To the accomplishment of the foregoing and related ends, this invention consists of features which will be hereinafter fully described, and particularly pointed out in the claims, the following description setting forth in detail certain embodiments of the invention, these being merely 20 illustrative of the principle of the present invention.

Broadly stated, this invention is directed to the use, in lubricants, of reaction products obtained by reacting organic compounds with hydrogen sulfide in the presence of ammonium hydrosulfide, and then treating said reaction products with phosphorus and halogen containing agents, such as the phosphorus halides and phosphorus oxyhalides and the like. Among the organic compounds which can be used to form reaction products of this invention are:

#### I. ALIPHATIC HYDROCARBONS

##### *Acyclic compounds*

A. Saturated paraffinic hydrocarbons above 6 carbon atoms such as

hexane  
heptane  
octane  
nonane  
tetradecane  
hexadecane  
eicosane  
tetracosane and the like.

B. Unsaturated paraffinic hydrocarbons above 6 carbon atoms such as

hexylene  
heptylene  
polyolefines

which may be broadly termed polyalkenes, and include polypropene, polypentenes as 60 well as branched chain unsaturated hydrocarbons such as iso-olefines and iso-polyolefines.

##### *Cyclic compounds*

A. Saturated

cyclobutane  
cyclohexane  
cyclo-octane and the like.

B. Unsaturated

cyclopentadiene  
cyclohexene  
cyclo-octene and the like.

#### II. AROMATIC HYDROCARBONS

- A. benzene
- naphthalene
- anthracene
- phenanthrene
- bi-phenyl
- di-phenylmethane
- stilbene and the like.
- B. alkyl
- hydroxy
- amine
- nitro
- nitroso
- halogen
- carboxyl
- mercaptan
- substituted aromatic compounds of group IIA and the like.

#### III. CYCLIC TERPENES

cymene  
limonene  
pinene  
bornylene  
methene  
terpinolene  
terpin  
menthol  
menthone  
isoborneol  
camphor

#### IV. HETEROCYCLIC COMPOUNDS

furan  
furfural  
furfuryl alcohol  
furoic acid  
pyrone  
pyridine  
picolinic acid  
nicotinic acid  
pyran  
morpholine  
courarone and the like.

Both the cyclic terpenes and the heterocyclic compounds can have attached thereto substituent radicals, such as alkyl and alkenyl radicals, hydroxy and halogen groups, and the like.

#### V. ALCOHOLS

50 A. Aliphatic (saturated and unsaturated)

amyl alcohol  
hexyl alcohol  
heptyl alcohol  
octyl alcohol  
decyl alcohol  
dodecyl alcohol  
octadecyl alcohol  
carnaubyl alcohol  
oleyl alcohol

##### Polyhydric aliphatic alcohols

glycols  
pinocols  
erythrol  
mannitol

sorbitol and the like.

B. Aromatic alcohols

phenyl ethyl alcohol  
phenyl octyl alcohol  
octadecyl benzyl alcohol  
benzyl alcohol and the like.

C. Cyclic alcohols

naphthenic alcohol

## D. Natural occurring alcohols and synthetic alcohols

Alcohols as found in wool fat, sperm oil  
Alcohols produced by oxidation of hydrocarbons, e. g.

paraffin wax  
sweat wax  
petrolatum and the like.

## VI. PHENOLIC COMPOUNDS

phenol  
alkyl phenol  
catechol  
resorcinol  
pyrogallol

All of these compounds may contain substituent groups such as alkyl radicals, amino, halogen, carboxyl and the like, hydroquinone, quinone, orcinol, phloroglucinol, cresols, thymol, saligenin, cinnamyl alcohol, methyl phenyl carbinol, eugenol, cardanols, etc.

## VII. ACIDS

## A. Aliphatic (mono and polycarboxylic and hydroxy substituted acids and the like)

capric  
undecylic  
lauric  
myristic  
palmitic  
stearic  
arachidic acids;  
acrylic  
sorbic  
oleic  
linoleic  
linolinic acids;  
hydroxy stearic  
di and tri hydroxy stearic  
ricinoleic acids;  
alkyl malonic acid  
alkyl succinic acid  
alkyl glutaric acid  
glycolic acid  
pyruvic acid  
phthalonic acid  
lactic acid  
alkyl maleic acid  
alkyl malic acid  
alkyl tartaric acid  
alkyl citric acid  
keto acids  
suberic acid  
alkyl adipic acid  
tartronic acid and the like, acids produced by oxidation of hydrocarbon e. g.  
paraffin wax and the like.

## B. Aromatic acids

benzoic  
salicylic  
cinnamic  
hydrocinnamic  
phthalic  
naphthoic  
abietic  
aromatic and sulfonic acids derived from petroleum hydrocarbons, mandelic acid, and the like;  
phenyl acetic acid  
phenyl stearic acid  
naphthyl stearic acid  
resinic acid

Both the aromatic and aliphatic acids of group VII can have attached thereto substituent groups as suggested under groups II, III, and IV.

## VIII. ESTERS

Esters contemplated for use in this invention may be obtained by reactioning any of the compounds listed under group V and VI and their derivatives, with any of the acids listed under group VII.

## IX. ETHERS

The ethers contemplated for use in this invention may be symmetrical, unsymmetrical, or mixed ethers of dialkyl ethers, alkyl-aryl ethers, aryl ethers and the like. Specifically it is desirable to use:

## X. ETHERS

## A. Aliphatic (saturated and unsaturated)

20 ethyl vinyl ether  
ethyl propenyl ether  
methyl isopropenyl ether  
ethyl isopropenyl ether  
methylallyl ether  
ethyl allyl ether  
n-propyl allyl ether  
isopropyl allyl ether  
4-ethoxy-1-butene  
6-ethoxy-1-hexene  
ethyl propargyl, etc.  
divinyl ether, diallyl ether  
dicrotonyl ether, dimethylallyl ether  
di-isopropenyl ether  
di(alpha-methylallyl) ether  
(1-butene-3-yl) (2-butene-4-yl) ether  
dihexaryl ether  
allyl (2-methyl-4-pentene-2-yl) ether  
allyl linanyl ether

## B. Cyclic and poly ethers

40 ethylene oxide  
propylene oxide  
acetal  
dioxan and the like.

## C. Aromatic ethers

allyloxyphenyl ether  
anisole, phenetole, diphenyl, dixenyl, di-naphthyl ethers  
benzyl phenyl ether  
cardanoxyethanol  
benzyl ether  
allyl-alpha phenyl vinyl ether  
allyl phenyl ether and the like.

## D. Substituted ethers

alkyloxy ethers of polyhydroxy aromatics such as resorcinol, pyrogallol, and the like.

## XI. ALDEHYDES

## A. Aliphatic (saturated and unsaturated)

60 acetaldehyde  
propionaldehyde  
butyraldehyde  
caproaldehyde and the like;  
acrolein  
crotonaldehyde  
citraal, etc.

## B. Aromatic

benzaldehyde  
cinnamaldehyde  
salicylaldehyde  
naphthaldehyde  
vanillin, etc.

## XII. KETONES

## A. Aliphatic (saturated and unsaturated)

acetone, butanone, hexanone, oleone, palmitone, methyl ethyl ketone, methyl propyl ketone, butyrone, butenone, pentanone, phorone, pentanedione, mesityl oxide, diethyl ketone, 3-methyl-heptanone, di-isobutyl ketone, diacetone alcohol, and the like.

## B. Aromatic

acetophenone  
propiophenone  
dibenzyl ketone  
benzyl phenyl ketone  
benzophenone and the like.

## C. Cyclic ketones

cyclobutanone, cyclohexanone, carvo-  
menthone, menthone, cyclopentanone  
pulegone, carvone, muscone, quinones,  
cycloheptanone, pure isophorone, and  
isophorone bottoms the manufacture of  
which will be fully described herein-  
after.

XIII. NATURAL FATS, OILS AND WAXES  
AND THEIR DERIVATIVES AND MISCELLANEOUS COMPOUNDSA. Vegetable and animal oils, fats, and waxes  
such as:

|                 |                         |
|-----------------|-------------------------|
| castor oil      | whale oil               |
| cocoanut oil    | wool fat                |
| corn oil        | Japan wax               |
| cottonseed oil  | olefin waxes            |
| horse fat       | paraffin waxes          |
| lard oil        | wax tailings            |
| mutton tallow   | petrolatum              |
| beef tallow     | vegetable and animal    |
| neat's-foot oil | phosphatidic materials  |
| palm oil        | montan wax              |
| peanut oil      | carnauba wax            |
| rapeseed oil    | beeswax                 |
| soya bean oil   | spermaceti              |
| sperm oil       | castor oil distillate   |
|                 | ozokerite               |
|                 | tall oil, and the like. |

## B. Petroleum hydrocarbons such as:

naphtha  
mineral seal oil  
kerosene  
gas oils, etc.

XIV. Metal salts and organic bases of organic  
materials listed in any of the above groups, their  
mixtures, or various combinations may be treated  
with hydrogen sulfide in presence of ammonium  
hydrosulfide and thereafter reacted with a  
phosphorus-halogen containing agent. Metal  
bases include those of the alkali metals, Cu, Mg,  
Ca, Ba, Zn, Cd, Al, Sn, Pb, Cr, Mn, Fe, Ni, Co,  
etc. Organic bases include various nitrogen bases  
as primary, secondary, tertiary and quaternary  
amines.

Among the specific and preferred compounds  
contemplated for reacting with hydrogen sulfide  
in the presence of ammonium hydrosulfide and  
further treating said product with a phosphorus  
and halogen containing agent, may be men-  
tioned: stilbene, oleic acid, ammonium oleate,  
potassium oleate, ammonium undecylenate, ethyl

undecylenate, methyl ricinoleate, cottonseed oil,  
rapeseed oil, peanut oil, dehydrated castor oil,  
and tall oil as well as wax olefins, cinnamyl alco-  
hol, pentanedione-2,4-diphenyl methane, high  
molecular weight saturated and unsaturated ketones,  
diacetone alcohol, mesityl oxide, ethyl  
oleate, ethyl cinnamate, cinnamaldehyde, and  
isophorone bottoms, the production and identi-  
fication of which latter will be fully described  
below.

Isophorone bottoms are primarily high molec-  
ular weight unsaturated ketones having at least  
12 and preferably more than 18 carbon atoms in  
the molecule. These products may be obtained  
15 by condensation of acetone in a caustic solution  
under elevated temperature and pressure. Spec-  
ifically the product is obtainable by condensing  
acetone in a 30% to 60% caustic solution at a  
temperature ranging between about 130° C. and  
about 170° C., and under a pressure of from about  
300 to about 500 pounds per square inch. The  
resultant product is subjected to distillation to re-  
move distillable ketones and other constituents  
and impurities. The product remaining in the  
still is preferably purified by filtration, solvent  
25 treatment, and comprises crude unsaturated  
cyclic ketones of high molecular weight, prefer-  
ably referred to as "crude isophorone bottoms."  
The term "isophorone bottoms" as referred to  
herein is usually a complex mixture of high molec-  
ular weight unsaturated cyclic ketones containing  
at least 12 and preferably more than 18 carbon  
atoms in the molecule. The product thus formed  
is not to be confused with straight isophorone  
35 which is specifically 3,5,5-trimethyl cyclohexene-  
2-one-1, which is an unsaturated cyclic ketone  
containing only nine carbon atoms in the molec-  
ule. Isophorone bottoms produced by condensa-  
tion of acetone under conditions referred to above  
40 includes within its scope any and all unsaturated  
cyclic ketones containing at least 12 and prefer-  
ably more than 18 carbon atoms and having gen-  
erally the chemical structural configuration of  
isophorone as well as the chemical structural  
45 configuration resulting from its further condensa-  
tion.

Crude isophorone bottoms can be fractionated  
and/or chemically treated and each fraction  
therefrom can in turn be treated with phosphorus  
halide at elevated temperatures to produce reac-  
tion products containing both phosphorus and  
50 halogen. Among the various fractions which can  
be obtained from crude isophorone bottoms are  
topped, crude isophorone bottoms which contain  
at least 18 carbon atoms in the molecule and are  
55 obtained after removal of distillate from crude  
isophorone bottoms to a still head temperature  
of 140° C. at 10 mm. mercury pressure. Another  
fraction of crude isophorone bottoms can be sub-  
jected to hydrolysis with dilute sodium hydroxide  
60 and the acetone and isophorone formed removed  
by distillation. The bottoms can then be filtered  
and purified and comprise essentially unsaturated  
cyclic ketones containing at least 12 and more  
65 carbon atoms in the molecule and are referred  
to as crude, hydrolyzed isophorone bottoms.  
This material can be subjected to distillation to  
split it into two fractions. The distilled hydro-  
lyzed isophorone fraction has a boiling point of  
70 about 140° C. at 10 mm. mercury pressure and  
consists of a mixture of unsaturated cyclic ketones  
containing between 15 to 18 carbon atoms in the  
molecule. The residue is referred to as topped,  
75 crude hydrolyzed isophorone bottoms and is  
similar to topped crude isophorone bottoms.

This residue comprises essentially unsaturated cyclic ketones of at least 15 carbon atoms and higher in the molecule. Crude isophorone bottoms can be also subjected to condensation over solid sodium hydroxide to yield two types of resinous materials. The first resinous fraction or soft resin has a viscosity at 210° F. of about 25-26 centistokes and an average molecular weight of from 320 to 350. The heavier fraction or medium resin has a viscosity at 210° F. of about 25-26 centistokes and an average molecular weight of from 320 to 350. The heavier fraction or medium resin has a viscosity at 210° F. of about 80 to 120 centistokes and an average molecular weight of from 370 to 390. The unsaturated cyclic ketones can be hydrogenated to produce saturated cyclic ketones. All of the various saturated and unsaturated cyclic ketone fractions obtained in the manner described above can be used. All of the various saturated and unsaturated cyclic ketone fractions obtained in the manner described above can, in accordance with one phase of this invention, be first reacted with hydrogen sulfide in the presence of ammonium hydrosulfide and the reaction product thus formed may then be further treated with a phosphorus halide to form desired final reaction products having outstanding properties as improving agents for lubricants. Among the phosphorus halides which can be used to treat the initial reaction, namely the reaction of hydrogen sulfide-ammonium hydrosulfide and an organic compound are:  $\text{PCl}_3$ ,  $\text{PCl}_5$ ,  $\text{PFBr}_2$ ,  $\text{PBr}_3$ ,  $\text{POBr}_3$ ,  $\text{POCl}_3$ ,  $\text{POF}_3$ ,  $\text{POFCl}_2$ ,  $\text{POFBr}_2$ ,  $\text{POF}_2\text{Cl}$ ,  $\text{POF}_2\text{Br}$ ,  $\text{P}_2\text{O}_3\text{Cl}_4$ ,  $\text{PO}_2\text{Cl}$ ,  $\text{PCl}_2\text{Br}$ ,  $\text{PSCl}_3$ ,  $\text{PI}_3$ ,  $\text{P}_2\text{I}_4$  and the like.

In carrying out the final reaction product it is preferable to do it in the presence of a peroxide catalyst which may include: hydrogen peroxide, benzoyl peroxide, lauroyl peroxide, tetratin peroxide, urea peroxide, butyl peroxide, diethyl peroxide, di-tert-butyl peroxide, diacyl peroxide, acetyl benzoyl peroxide, propionyl peroxide, cyclohexanone peroxide, ascaridole, alkali and alkaline earth metal peroxides or mixtures thereof can be used.

The products formed by the reaction of hydrogen sulfide-ammonium hydrosulfide with an organic compound can be prepared at room or elevated temperatures, preferably in closed vessels. The use of elevated temperatures apparently only speeds up the reaction. However, the cost of fuel and special equipment outweighs this feature, and it has been ordinarily found more advantageous to simply allow the ammonium hydrosulfide-hydrogen sulfide organic compound reactions to take place at room temperature in closed vessels for the necessary period of time, e. g. from one week to one month or more, depending upon the organic material being treated. The final reaction product which is formed by treating the reaction products of ammonium hydrosulfide-hydrogen sulfide and an organic compound with any of the previously mentioned phosphorus halides can be carried out at elevated temperatures of between about 100° C. and about 200° C. and preferably between about 150° C. and about 170° C. and if desired in the presence of a suitable inert solvent and a peroxide catalyst.

To more clearly illustrate the present invention, the following examples are presented. It is to be understood however that various modifications can be resorted to without departing from the spirit of the invention.

## EXAMPLE I

## A. Initial reaction product of hydrogen sulfide in the presence of ammonium hydrosulfide with topped, crude isophorone bottoms

Isopropyl alcohol (700 cc.) contained in a 4-liter, thick-walled suction flask, was saturated with dry ammonia followed by dry hydrogen sulfide. A solution of 238.5 grams of topped, crude isophorone bottoms in 350 cc. isopropyl alcohol was added and the resulting solution was saturated with hydrogen sulfide. The side-neck and mouth of the flask were then closed and the flask was allowed to stand for a week with infrequent shaking. Upon opening the flask a partial vacuum was discovered. The reaction mixture was filtered to remove impurities and the isopropyl alcohol was removed from the filtrate by evaporation. The residue was dissolved in 500 cc. of a non-aromatic hydrocarbon having a boiling range of between about 164° F. and 233° F. and washed with water. After removal of the solvent in a current of nitrogen gas on a steam bath, a very viscous sticky mass was obtained, said mass possessing a pleasant odor and exhibiting much less flow at room temperature than did the starting materials. The product was oil-soluble and on analysis contained:

|    | Analysis of Product                                                    | Analysis of cyclic ketone (topped, crude isophorone bottom) |
|----|------------------------------------------------------------------------|-------------------------------------------------------------|
| 30 |                                                                        |                                                             |
| 35 | Per cent by wt. Sulfur.....                                            | 7.2 (5)                                                     |
|    | Per cent by wt. Carbon.....                                            | 76.2 (1)                                                    |
|    | Per cent by wt. Hydrogen.....                                          | 9.6 (2)                                                     |
|    | Per cent by wt. Nitrogen.....                                          | 0.26                                                        |
|    | Per cent by wt. Oxygen (by difference).....                            | 6.6 (6)                                                     |
| 40 | Mol. wt. (ebullioscopic determination in $\text{C}_6\text{H}_6$ )..... | 352                                                         |
|    |                                                                        | 316                                                         |

## B. Final reaction product obtained by treating (A) with phosphorus pentachloride

To approximately 170 grams of the above initial reaction product about 450 grams of phosphorus pentachloride and about 3.2 grams of di-tert-butyl peroxide were admixed in a suitable vessel and the mixture was heated and stirred on a steam bath for about 24 hours. At the end of the reaction period, the desired product was extracted with a non-aromatic hydrocarbon having a boiling range of between about 164° F. and 233° F. The solution was filtered and the filtrate evaporated at steam temperature in a current of carbon dioxide. The resultant product was a viscous mass containing a substantial amount of sulfur, phosphorus and chlorine.

## EXAMPLE II

## A. Initial reaction product of ammonium hydrosulfide-hydrogen sulfide and topped, crude isophorone bottoms

This reaction product was prepared in an isopropyl alcohol medium (1315 cc.) using about 295 gm. of topped, crude isophorone bottoms in an autoclave for 5½ hours at 96° C. to 101.5° C. The product was then treated as indicated in Example I, part A, and the analysis of the product was as follows:

|    |                                |          |
|----|--------------------------------|----------|
| 70 | Per cent by wt. sulfur .....   | 6.2      |
|    | Per cent by wt. carbon .....   | 77.2 (3) |
|    | Per cent by wt. hydrogen ..... | 9.6 (2)  |
|    | Per cent by wt. nitrogen ..... | 0.3 (9)  |
|    | Per cent by wt. oxygen .....   | 6.5 (6)  |
| 75 | Mol. wt. ....                  | 356      |

B. Final reaction product obtained by treating  
IIA with phosphorus oxychloride

To approximately 160 grams of the reaction product of IIA, about 306 grams of phosphorus oxychloride and about 3.2 grams of di-tert butyl peroxide were reacted as disclosed under IB. After removal of the extraction solvent and excess phosphorus oxychloride in *vacuo*, a dark residue remained which contained a substantial amount of sulfur, phosphorus and chlorine.

Other phosphorus halide treated ammonium hydrosulfide - hydrogen sulfide - organic compound reaction products which are particularly preferable as lubricating oil additives are as follows:

(1) Ammonium hydrosulfide-hydrogen sulfide-mesityl oxide treated with some phosphorus pentachloride or phosphorus oxychloride.

(2) Ammonium hydrosulfide-hydrogen sulfide-diacetone alcohol treated with some phosphorus pentachloride or phosphorus oxychloride.

(3) Ammonium hydrosulfide-hydrogen sulfide-wax olefins treated with some phosphorus pentachloride or phosphorus oxychloride.

(4) Ammonium hydrosulfide-hydrogen sulfide-stilbene treated with phosphorus pentachloride or phosphorus oxychloride.

(5) Ammonium hydrosulfide-hydrogen sulfide-pentadione-2,4 treated with some phosphorus pentachloride or phosphorus oxychloride.

(6) Ammonium hydrosulfide-hydrogen sulfide-diphenyl methane treated with some phosphorus pentachloride or phosphorus oxychloride.

(7) Ammonium hydrosulfide-hydrogen sulfide-oleic acid treated with some phosphorus pentachloride or phosphorus oxychloride.

(8) Ammonium hydrosulfide-hydrogen sulfide-ammonium oleate treated with some phosphorus pentachloride or phosphorus oxychloride.

(9) Ammonium hydrosulfide-hydrogen sulfide-potassium oleate treated with some phosphorus pentachloride or phosphorus oxychloride.

(10) Ammonium hydrosulfide-hydrogen sulfide-ammonium undecylenate treated with phosphorus pentachloride or phosphorus oxychloride.

(11) Ammonium hydrosulfide-hydrogen sulfide-ethyl undecylenate treated with phosphorus pentachloride or phosphorus oxychloride.

(12) Ammonium hydrosulfide-hydrogen sulfide-ethyl cinnamate treated with some phosphorus pentachloride or phosphorus oxychloride.

(13) Ammonium hydrosulfide-hydrogen sulfide-methyl ricinoleate treated with some phosphorus pentachloride or phosphorus oxychloride.

(14) Ammonium hydrosulfide-hydrogen sulfide-cottonseed oil treated with some phosphorus pentachloride or phosphorus oxychloride.

(15) Ammonium hydrosulfide-hydrogen sulfide-rapeseed oil treated with some phosphorus pentachloride or phosphorus oxychloride.

(16) Ammonium hydrosulfide-hydrogen sulfide-peanut oil treated with some phosphorus pentachloride or phosphorus oxychloride.

(17) Ammonium hydrosulfide-hydrogen sulfide-dehydrated castor oil treated with some phosphorus pentachloride or phosphorus oxychloride.

(18) Ammonium hydrosulfide-hydrogen sulfide-tall oil treated with some phosphorus pentachloride or phosphorus oxychloride.

(19) Ammonium hydrosulfide-hydrogen sulfide-cinnamyl alcohol treated with some phosphorus pentachloride or phosphorus oxychloride.

(20) Ammonium hydrosulfide-hydrogen sulfide-cinnamaldehyde treated with some phosphorus pentachloride or phosphorus oxychloride.

The herein described reaction products when added in small amounts to base lubricants are effective in inhibiting the formation of harmful deposits, corrosive materials, detrimental oxidation products and the like. They are also effective in imparting to lubricants to which they are added, extreme pressure, anti-wear, anti-ring-sticking corrosion inhibiting characteristics and the like.

In addition to the above properties the addition of reaction products of this invention to mineral lubricating oils inhibits lacquer formation in engines operating under the most adverse conditions. Also reaction products of this invention can be used as valuable constituents of heavy duty oils, motor oils, diesel oils, aviation oils, turbine oil, synthetic oils and the like because of their anti-corrosion, anti-oxidation, and anti-wear properties. Besides their utility as lubricating oil additives, reaction products of this invention are useful as anti-oxidants for natural and synthetic rubber and other organic materials which are subject to oxidation deterioration. The amount of additive used can be varied over wide limits but generally it is not necessary to use more than 5% by weight of the reaction product and preferably only between about 0.1 to 2.0% by weight is added to base lubricants.

Because of its synergistic effect the reaction product of this invention can be combined with other additives in lubricants, such as blooming agents, pour point depressants or viscosity improvers, extreme pressure agents, anti-foaming agents and the like. Among the specific additives which can be used are oil-soluble detergents which include oil-soluble salts of various bases with detergent forming acids. Such bases include metal as well as organic bases. Metallic bases include those of the alkali metals, Cu, Mg, Ca, Sr, Ba, Zn, Cd, Al, Sn, Pb, Cr, Mn, Fe, Ni, Co, etc. Organic bases include various nitrogen bases as primary, secondary, tertiary and quaternary amines.

Examples of detergent forming acids are the various fatty acids of, say 10 to 30 carbon atoms, wool fat acids, paraffin wax acids (produced by oxidation of paraffin wax) chlorinated fatty acids, rosen acids, aromatic carboxylic acids including aromatic fatty acids, aromatic hydroxy fatty acids, paraffin wax benzoic acids, various alkyl salicylic acids, phthalic acid monoesters, aromatic keto acids, aromatic ether acids, diphenols as di-(alkylphenol) sulfides and disulfides, methylene bis alkylphenols, sulfonic acids such as may be produced by treatment of alkyl aryl hydrocarbons or high boiling petroleum oils with sulfuric acid; sulfuric acid; sulfuric acid monoesters; phosphoric, arsonic and antimony acid mono and diesters, including the corresponding thio-phosphoric, arsonic and antimony acids; phosphonic and arsonic acids and the like.

Additional detergents are the alkaline earth phosphate diesters, including the thiophosphate diester; the alkaline earth diphenolates, specifically the calcium and barium salts of diphenol mono and poly sulfides.

Non-metallic detergents include compounds such as the phosphatides such as lecithin and caphlin, certain fatty oils as rapeseed oils, 75 volatilized fatty or mineral oils and the like.

An excellent metallic detergent for the present purpose is the calcium salt of oil-soluble petroleum sulfonic acids. This may be present advantageously in the amount of about 0.025% to 0.2% sulfate ash. Also alkaline metal salts of alkyl phenol-aldehyde condensation reaction products are excellent detergents.

Anti-oxidants comprise several types, for example, alkyl phenols such as 2,4,6-trimethyl phenol, pentamethyl phenol, 2,4-dimethyl-6-tertiary-butyl phenol, 2,4-dimethyl-6-octyl phenol, 2,6-di-tertiary-butyl-4-methyl-phenol, 2,4,6-tri-tertiary-butyl phenol and the like; amino phenols as benzyl amino phenols; amines such as dibutyl phenylene diamine, diphenyl amine, phenyl - beta - naphthylamine, phenyl - alpha - naphthylamine, dinaphthyl amine.

Corrosion inhibitors or anti-rusting compounds may also be present, such as dicarboxylic acids of 16 and more carbon atoms; alkali metal and alkaline earth salts of sulfonic acids and fatty acids; organic compounds containing an acidic radical in close proximity to a nitrile, nitro or nitroso group (e. g. alpha cyano stearic acid).

Extreme pressure agents which may be used comprise: esters of phosphorus acids such as triaryl, alkyl hydroxy aryl, or aralkyl phosphates, thio-phosphates or phosphites and the like; neutral aromatic sulfur compounds of relatively high boiling temperatures such as diaryl sulfides, diaryl disulfides, alkyl aryl disulfides, e. g. diphenyl sulfide, diphenol sulfide, diresol sulfide, dixylenol sulfide, methyl butyl diphenol sulfide, dibenzyl sulfide, corresponding di- and tri-sulfides, and the like; sulfurized fatty oils or esters of fatty acids and monohydric alcohols, e. g. sperm oil, jojoba oil, etc.; in which the sulfur is strongly bonded; sulfurized long chain olefins such as may be obtained by dehydrogenation or cracking of wax; sulfurized phosphorized fatty oils or acids, phosphorus acid esters having sulfurized organic radicals, such as esters of phosphoric or phosphorus acids with sulfurized hydroxy fatty acids; chlorinated hydrocarbons, such as chlorinated paraffin, aromatic hydrocarbons, terpenes, mineral lubricating oil, etc.; or chlorinated esters of fatty acids containing the chlorine in position other than alpha position.

Additional ingredients may comprise oil-soluble urea or thiourea derivatives, e. g. urethanes, allophanates, carbazides, carbazones, etc.; polyisobutylene polymers, unsaturated polymerized esters of fatty acids and monohydric alcohols and other high molecular weight oil-soluble compounds.

Depending upon the additive used and conditions under which it is used, the amount of additive used may vary from 0.01 to 2% or higher. However, substantial improvement is obtained by using amounts ranging from 0.1 to 0.5% in combination with phosphorous sulfide-unsaturated cyclic ketone reaction product of this invention.

It is to be understood that while the features of the invention have been described and illustrated in connection with certain specific examples, the invention, however, is not to be limited thereto or otherwise restricted, except by the prior art and the scope of the appended claims.

This application is a continuation-in-part of the co-pending application, Serial No. 718,617, filed December 26, 1946, which has matured into U. S. Patent 2,512,784.

I claim as my invention:

1. A lubricant comprising a major amount of

a lubricating oil and a minor amount, sufficient to stabilize said oil against oxidation and corrosion deterioration, of a reaction product obtained by reacting an unsaturated cyclic ketone fraction having at least 12 carbon atoms with hydrogen sulfide and ammonium hydrosulfide, at between about room temperature and about 100° C. and treating the resulting reaction product with a phosphorus halide at between about steam temperature and 200° C. in the mol ratio of around 1 to 4 respectively.

2. A lubricant comprising a major amount of mineral lubricating oil and a minor amount, of from 0.1% to 5% by weight, of a reaction product obtained by reacting an unsaturated cyclic ketone fraction having at least 12 carbon atoms with hydrogen sulfide and ammonium hydrosulfide at between about room temperature and 100° C. and treating the resulting reaction product with phosphorus pentachloride at a temperature of at least 150° C. in the mol ratio of around 1 to 4 respectively.

3. A lubricant comprising a major amount of mineral lubricating oil and a minor amount, of from 0.1% to 5% by weight, of a reaction product obtained by reacting isophorone bottoms fraction having at least 12 carbon atoms with hydrogen sulfide and ammonium hydrosulfide at between about room temperature and 100° C. and treating the resulting reaction product with phosphorus pentachloride at a temperature of at least 150° C. in the mol ratio of around 1 to 4 respectively.

4. A lubricant comprising a major amount of mineral lubricating oil and a minor amount, of from 0.1% to 5% by weight, of a reaction product obtained by reacting an unsaturated cyclic ketone fraction having at least 12 carbon atoms with hydrogen sulfide and ammonium hydrosulfide at between about room temperature and 100° C. and treating the resulting reaction product with phosphorus oxychloride at a temperature of at least 150° C. in the mol ratio of around 1 to 4 respectively.

5. A lubricant comprising a major amount of mineral lubricating oil and a minor amount, of from 0.1% to 5% by weight, of a reaction product obtained by reacting isophorone bottoms fraction having at least 12 carbon atoms with hydrogen sulfide and ammonium hydrosulfide at between about room temperature and 100° C. and treating the resulting reaction product with phosphorus oxychloride at a temperature of at least 150° C. in the mol ratio of around 1 to 4 respectively.

55. 6. A compounded lubricant comprising a major amount of a mineral lubricating oil and containing an active amount of calcium salt of alkyl phenol-formaldehyde condensation reaction product, calcium salt of petroleum sulfonic acid as detergents, and a small amount of from 0.1% to 5% by weight of a reaction product obtained by reacting an unsaturated cyclic ketone fraction having at least 12 carbon atoms with hydrogen sulfide and ammonium hydrosulfide, at between about room temperature and about 100° C. and treating the resulting reaction product with a phosphorus halide at a temperature of at least 150° C. in the mol ratio of around 1 to 4 respectively.

70. 7. An organic composition having incorporated therein as the essential stabilizing agent the reaction product obtained by first reacting an unsaturated cyclic ketone fraction having at least 12 carbon atoms with hydrogen sulfide and ammonium hydrosulfide at between about room

15

temperature and 100° C. and treating the resulting reaction product with phosphorus pentachloride at a temperature of at least 150° C. in the mol ratio of around 1 to 4 respectively.

16. An organic composition having incorporated therein as the essential stabilizing agent the reaction product obtained by first reacting an unsaturated cyclic ketone fraction having at least 12 carbon atoms with hydrogen sulfide and ammonium hydrosulfide at between about room temperature to 100° C. and treating the resulting reaction product with phosphorus pentachloride at between about room temperature and 200° C. in the mol ratio of around 1 to 4 respectively.

17. As a composition, the reaction product obtained by first reacting an unsaturated cyclic ketone fraction having at least 12 carbon atoms with hydrogen sulfide and ammonium hydrosulfide at between about room temperature and 100° C. and treating the resulting reaction product with phosphorus halide at a temperature of at least 150° C. in the mol ratio of around 1 to 4 respectively.

18. A compounded lubricant comprising a major amount of a mineral lubricating oil and containing an active amount of calcium salt of alkyl phenol-formaldehyde condensation reaction product; calcium salt of petroleum sulfonic acid

as detergents and a small amount of from 0.1% to 5% by weight of a reaction product obtained by reacting isophorone bottoms fraction having at least 12 carbon atoms with hydrogen sulfide and ammonium hydrosulfide at between about room temperature and 100° C. and treating the resulting reaction product with phosphorus pentachloride at a temperature of at least 150° C. in the mol ratio of around 1 to 4 respectively.

19. As a composition, the reaction product obtained by first reacting isophorone bottoms fraction having at least 12 carbon atoms with hydrogen sulfide and ammonium hydrosulfide at between about room temperature and 100° C. and treating the resulting reaction product with phosphorus pentachloride at a temperature of at least 150° C. in the mol ratio of around 1 to 4 respectively.

DAVID E. ADELSON.

## REFERENCES CITED

The following references are of record in the file of this patent:

## UNITED STATES PATENTS

| Number    | Name     | Date          |
|-----------|----------|---------------|
| 2,382,121 | Whittler | Aug. 14, 1945 |
| 2,413,648 | Ott      | Dec. 31, 1946 |